

## UNITED STATES PATENT OFFICE.

SAMUEL S. SADTLER, OF SPRINGFIELD TOWNSHIP, MONTGOMERY COUNTY, PENNSYLVANIA, ASSIGNOR TO AMIESITE ASPHALT COMPANY OF AMERICA, OF PHILADELPHIA, PENNSYLVANIA, A CORPORATION OF NEW JERSEY.

## ART OF ROAD MAKING.

No Drawing.

Application filed March 26, 1927. Serial No. 178,814.

This invention relates to improvements in the art of roadmaking, and the principal object of the invention is to provide novel and improved means for coating damp stone, 5 constituting the aggregate of which the road composition is made, with asphalt or other bitumen.

Another object of the invention is to provide a novel and improved method particularly applicable to the coating of limestone and stone of like alkaline nature.

It is frequently desirable to make roadways of the general type set forth in U. S. Patent No. 1,611,444, without special drying 15 of the stone of the aggregate in preparation for coating the stone with bitumen. Difficulty, however, has been experienced in the absence of the drying operation of obtaining a satisfactory bond between the bitumen 20 and the surfaces of the stone. It has been particularly difficult to obtain satisfactory results under the stated circumstances in connection with roadways or surfaces in which the voids between the bitumen-coated 25 stones are not filled and in which the stones are cemented together solely or principally by their asphaltic or bitumen coatings.

With certain stones of dense character in which ferro magnesium minerals predominate, such for example as gabbro or basalt, 30 light hydrocarbon oils such as kerosene and naphtha and bitumens such as asphalt derived from petroleum have a preferential affinity for the stone surfaces even when the 35 surfaces are somewhat damp. For minerals of this character, I find it sufficient to add light hydrocarbon oils of a slowly volatile nature, such as kerosene, to the aggregate; and after agitation, in a pug mill for ex- 40 ample, it will be found that the kerosene or other liquefier will displace whatever water there may be on the stone surfaces, and satisfactorily prepare the surfaces for reception 45 of the asphalt or other bitumen, which is then added. By this means a satisfactory coating can be obtained with the bitumen in intimate contact with the stone surfaces.

In this process I may use about one gallon 50 or one and one-half gallons of the liquefier, which as stated above may be kerosene or other slowly volatile light hydrocarbon oil,

to 1900 lbs. of stone. Preferably the stone is heated to a temperature between 60° and 90° F. To this liquefier-treated stone I then 55 add melted asphalt at a temperature of say 212° F. or slightly higher to the extent of about 80 to 100 lbs., depending upon the size of the stone and using less asphalt for stone of larger sizes such as would be used 60 for a base course, and larger quantities for stone of the smaller sizes such as may be used for the top or wearing course of the finished roadbed. After the asphalt has been thoroughly incorporated and spread 65 through the stones and over all the surfaces, I preferably add from 6 to 10 lbs. of hydrated lime, which is thoroughly distributed through the mass when the operation of coating is completed. 70

I have found, however, that certain types of stones, and particularly limestone, do not respond to the above process. Limestone when at all damp and often when containing as little as a few tenths of a percent 75 of moisture will not take a commercial coating of bitumen with the aforescribed procedure. Under some conditions, the asphalt may be spread over the surfaces of the stone with the use of a liquefier as described, but 80 it will not adhere and will have a tendency to peel off. Where such materials are used in roadways, the stones may actually become loose from one another and result in complete failure of the road surface. 85

I have discovered that by dissolving in the liquefier some form of soap containing unneutralized acids, the attraction of the bitumen or asphalt to stone of alkaline nature such as limestone is promoted, with 90 the result that a firm bond between the asphalt and stone surfaces is obtained. I prefer to use some form of sulfonated oil partly neutralized with ammonia, although simple organic acids such as oleic, partly 95 neutralized with ammonia, will be found satisfactory. In any case, the acid is only partially neutralized, and I prefer to use ammonia as the base for such neutralization, as ammonia is relatively more soluble in 100 hydrocarbon oils such as kerosene. Successful coatings have been made using five ounces to one lb. of oleic acid or sulfonated oil slightly neutralized with ammonia, the

procedure and the proportions of the other ingredients of the mix being substantially the same as those recited above.

I do not, however, limit myself to any particular quantities or proportions.

I claim:

1. The method of coating stone of alkaline nature, which consists in taking a bitumen liquefier such as kerosene, dissolving therein a soap containing unneutralized acid, treating the stone with the liquefier composition, and thereafter incorporating a bitumen.
- 10 2. The method of coating damp stone of alkaline nature, which consists in taking a bitumen liquefier to which has been added a soap containing unneutralized acid, said soap being soluble in the liquefier, treating
- 15

the stone with said mixture, and thereafter adding a bitumen.

3. The method of coating damp stone of 20 alkaline nature, which consists in taking a bitumen liquefier such as kerosene, adding thereto a sulfonated oil partly neutralized with ammonia and soluble in the liquefier, treating the stone with said mixture, and 25 thereafter incorporating a bitumen.

4. The method of coating damp stone of an alkaline nature, which consists in adding to a bitumen liquefier such as kerosene an organic acid such as oleic partly neutralized with ammonia and soluble in the liquefier, treating the stone with said mixture, and 30 thereafter incorporating a bitumen.

SAMUEL S. SADTLER.